

Oct. 19, 1954

T. H. INSINGER, JR.

2,692,234

## HEAT TRANSFER MEDIA

Filed Nov. 5, 1949



INVENTOR.  
THOMAS H. INSINGER, JR.

BY Edmund G. Borden

*his* ATTORNEY

## UNITED STATES PATENT OFFICE

2,692,234

## HEAT TRANSFER MEDIA

Thomas Harold Insinger, Jr., Sewickley, Pa., assignor to Koppers Company, Inc., Pittsburgh, Pa., a corporation of Delaware

Application November 5, 1949, Serial No. 125,802

2 Claims. (Cl. 252—71)

1

This invention relates to heat transfer media. More particularly the invention relates to high temperature heat transfer media which have solidification points below 140° C.

Many chemical reactions may be carried out more advantageously when the reaction products are heated to uniformly controlled temperatures. Some inorganic salts in molten state have been used as heat transfer media, but many of the molten salt solutions heretofore used for operating at temperatures between 400° and 500° C. have high solidification points which make them inconvenient to handle.

To permit the molten inorganic salt solutions to be safely used as heat transfer media, it is customary to circulate the media in a tightly closed circuit immersed in or enclosing the material to be heated and to circulate the molten salt solution in a closed cycle between a heat source and the reaction vessel, so that the heat is transferred through a diaphragm. If it becomes necessary to discontinue circulation of the molten salt solution and it is allowed to cool it will solidify. Since the molten salt solution generally fills most or all of the coil or circuit container, it is very difficult to again melt a high solidification temperature transfer media so that it may be again put into circulation.

The primary object of the present invention is to provide high temperature heat transfer media that have solidification points below 100° C. or the temperature of saturated steam at atmospheric pressure.

Another object of the invention is to provide high temperature heat transfer media that have solidification points below the temperature of moderate pressure dry steam, that is, the temperature of dry saturated steam at a gauge pressure of 50 pounds per square inch.

Another object of the invention is to provide a heating medium which is thermally stable and capable of transferring heat at a temperature above 450° C., and which has a relatively low melting point.

With these and other objects in view, the invention consists in the high temperature heat transfer media hereinafter described and particularly defined in the claims.

The heat transfer media of the present invention are ternary mixtures of lithium nitrate, potassium nitrate and sodium nitrite. These three inorganic salts form a ternary eutectic which does not solidify at temperatures above 70° C. and the media formed by different mixtures are capable of stable operation at temperatures above 450° C.

2

For example the following mixtures of three components mentioned above have the following solidification points, the composition of the components being expressed as percent by weight—

| Solidification Point, ° C. | Composition                 |                             |                            |
|----------------------------|-----------------------------|-----------------------------|----------------------------|
|                            | LiNO <sub>3</sub> , Percent | NaNO <sub>2</sub> , Percent | KNO <sub>3</sub> , Percent |
| 70                         | 22.0                        | 47.5                        | 30.5                       |
| 70                         | 23.0                        | 47.0                        | 30.0                       |
| 71                         | 25.0                        | 44.8                        | 30.2                       |
| 72                         | 16.0                        | 42.0                        | 42.0                       |
| 72                         | 16.0                        | 46.0                        | 38.0                       |
| 73                         | 16.0                        | 38.6                        | 45.4                       |
| 73                         | 17.5                        | 41.9                        | 40.6                       |
| 73                         | 13.0                        | 49.7                        | 37.3                       |
| 76                         | 15.0                        | 55.0                        | 30.0                       |
| 78                         | 10.0                        | 20.0                        | 70.0                       |
| 80                         | 30.0                        | 40.0                        | 30.0                       |
| 81                         | 10.0                        | 64.0                        | 26.0                       |
| 87                         | 13.0                        | 43.7                        | 43.3                       |
| 87                         | 29.0                        | 28.5                        | 42.5                       |
| 90                         | 21.0                        | 20.0                        | 59.0                       |
| 90                         | 25.0                        | 50.0                        | 25.0                       |
| 91                         | 10.0                        | 30.0                        | 60.0                       |
| 96                         | 70.0                        | 10.0                        | 20.0                       |
| 99                         | 54.0                        | 20.0                        | 26.0                       |
| 104                        | 60.0                        | 10.0                        | 30.0                       |
| 108                        | 40.0                        | 10.0                        | 50.0                       |
| 109.5                      | 6.0                         | 54.0                        | 40.0                       |
| 110                        | 40.0                        | 50.0                        | 10.0                       |
| 112                        | 6.0                         | 25.0                        | 66.0                       |
| 114                        | 6.0                         | 41.0                        | 53.0                       |
| 114                        | 70.0                        | 20.0                        | 10.0                       |
| 119                        | 50.0                        | 30.0                        | 20.0                       |
| 121                        | 60.0                        | 30.0                        | 10.0                       |
| 127                        | 22.0                        | 6.0                         | 72.0                       |
| 131                        | 2.0                         | 66.0                        | 32.0                       |
| 133                        | 2.0                         | 37.0                        | 62.0                       |
| 139                        | 10.0                        | 70.0                        | 20.0                       |
| 139                        | 20.0                        | 70.0                        | 10.0                       |
| 143                        | 10.0                        | 10.0                        | 80.0                       |
| 172                        | 2.0                         | 22.0                        | 76.0                       |

35 In the accompanying drawing the solidification points shown in the above table have been plotted on a chart of triangular coordinate paper which indicates the composition of each mixture (expressed as percent by weight) corresponding to 40 the solidification point of the mixture. A triangular plot is shown on the chart in dot-and-dash lines with one apex being a mixture composed of LiNO<sub>3</sub> 55%, NaNO<sub>2</sub> 20%, and KNO<sub>3</sub> 25%. Another apex is a mixture having a solidification temperature of 78° C. composed of LiNO<sub>3</sub> 10%, NaNO<sub>2</sub> 20% and KNO<sub>3</sub> 70%. A third apex is a mixture composed of LiNO<sub>3</sub> 10%, NaNO<sub>2</sub> 65% and KNO<sub>3</sub> 25%. All of the mixtures within the triangular area have solidification temperatures below 100° C. It is evident, however, that there could exist some mixtures having solidification temperatures of 100° C. or lower that would be outside, but close to the boundaries of the triangular plot. The majority of the mixtures 50 which have solidification temperatures between 70° and 100° C. are made up of LiNO<sub>3</sub> 10% to 55

55%,  $\text{NaNO}_2$  20% to 65%, and  $\text{KNO}_3$  25% to 70%. All of these mixtures which have solidification points below 100° C. are capable of operating as heating media at temperatures above 450° C.

It will be observed that compositions falling within the above described triangular plot but having not more than 30% lithium nitrate have the advantage of having the desired low solidification temperatures of between 70° and 100° C. and the further advantage that this result is obtained with less lithium nitrate, which is by far the most expensive ingredient, than needed to form the binary eutectic of lithium nitrate and potassium nitrate which has the lowest solidification point known in the art for any of the three components or mixtures thereof. Thus by replacing part of the relatively expensive ingredient, lithium nitrate, by sodium nitrite or sodium nitrite and potassium nitrate, compositions according to this invention are obtained which are substantially more economical and at the same time have markedly lower solidification points.

Below the triangular plot on the chart is a trapezoidal area of mixtures having solidification points from about 80° C. up to 140° C. The two upper corners of the trapezoid are first, a mixture composed of  $\text{LiNO}_3$  10%,  $\text{NaNO}_2$  25%, and  $\text{KNO}_3$  65%, and second a mixture having a solidification point of 139° C. composed of  $\text{LiNO}_3$  10%,  $\text{NaNO}_2$  70% and  $\text{KNO}_3$  20%. A third and lower corner is a mixture of  $\text{LiNO}_3$  2%,  $\text{NaNO}_2$  70% and  $\text{KNO}_3$  28%. The fourth and lower corner is a mixture compound of  $\text{LiNO}_3$  2%,  $\text{NaNO}_2$  25% and  $\text{KNO}_3$  73%. The mixtures within the trapezoidal area which have been examined all have solidification temperatures below 140° C. and are capable of operating as heating media at temperatures of 450° to 500° C.

Those mixtures of lithium nitrate, sodium nitrite and potassium nitrate which come within the area bounded by the dot-and-dash triangle are suitable for use as heat transfer media in an equipment which can be heated with saturated steam at atmospheric pressure or thereabouts to bring the heat transfer media into a liquid state for circulation in a closed heating cycle. The mixtures of lithium nitrate, potassium nitrate and sodium nitrite included in the trapezoidal area shown in the chart are preferably employed in apparatus which can be heated with dry saturated steam at a gauge pressure of 50 lbs. per square inch to prepare the heating media in condition for circulation in a closed heating cycle.

The eutectic temperature for a mixture of potassium nitrate and lithium nitrate has been

found to be 129° C. The eutectic temperature for a mixture of potassium nitrate and sodium nitrite has been found to be 139° C. It is believed that the eutectic temperature of a mixture of lithium nitrate and sodium nitrite has

not been accurately determined up to the present time. Lithium nitrate starts to decompose at about 475° C. Potassium nitrate has the decomposition temperature of 532.7° C. Sodium nitrite does not decompose to yield  $\text{NO}_2$  at temperatures below 600° C.

Any mixture of the components lithium nitrate, potassium nitrate and sodium nitrite as shown in the table and on the plot is capable of substantially stable operation at temperatures of 450° C. for an extended period of time. It will be understood however, that for high temperature operations the minimum amount of lithium nitrate is used on account of the cost of this component.

The preferred form of the invention having been thus described, what is claimed as new is:

1. A ternary mixture of approximately 16% by weight of lithium nitrate, 42% by weight of potassium nitrate, and 42% by weight of sodium nitrite.

2. A low solidification point fusible composition consisting of a ternary mixture of lithium nitrate, sodium nitrite and potassium nitrate having a percentage composition falling within the area on the chart of the drawing bounded substantially by the triangle formed by lines connecting the following points:

| $\text{LiNO}_3$ , Percent | $\text{NaNO}_2$ , Percent | $\text{KNO}_3$ , Percent |
|---------------------------|---------------------------|--------------------------|
| 25                        | 44.8                      | 30.2                     |
| 15                        | 55                        | 30                       |
| 16                        | 38.6                      | 45.4                     |

#### References Cited in the file of this patent

#### UNITED STATES PATENTS

| Number    | Name               | Date           |
|-----------|--------------------|----------------|
| 1,555,400 | Burns              | Sept. 29, 1925 |
| 1,984,369 | Gensch             | Dec. 18, 1934  |
| 2,148,664 | Wille et al.       | Feb. 28, 1939  |
| 2,205,180 | Shaver             | June 18, 1940  |
| 2,375,759 | Kalichevsky et al. | May 15, 1945   |
| 2,429,129 | Heppell et al.     | Oct. 14, 1947  |

#### FOREIGN PATENTS

| Number  | Country     | Date          |
|---------|-------------|---------------|
| 110,773 | Australia   | June 20, 1940 |
| 214,894 | Switzerland | Aug. 16, 1941 |